

Aug. 6, 1946.

C. C. HERITAGE

2,405,213

2,403,21  
PROCESS AND APPARATUS FOR PRODUCTION OF FIBER FROM VEGETABLE MATTER

Filed Aug. 3, 1940



Inventor  
Clark C. Heritage  
by W. Bartlett Jones,  
Attorney.

## UNITED STATES PATENT OFFICE

2,405,213

## PROCESS AND APPARATUS FOR PRODUCTION OF FIBER FROM VEGETABLE MATTER

Clark C. Heritage, Cloquet, Minn., assignor to  
Wood Conversion Company, Cloquet, Minn., a  
corporation of Delaware

Application August 3, 1940, Serial No. 351,066

5 Claims. (Cl. 92—6)

1

The present invention relates generally to the production of pulp, and in particular to apparatus therefor.

Reference is made to the Asplund U. S. Patent No. 2,008,892, describing a machine for the production of pulp. The raw material in the form of wood chips, grasses, straw, bagasse, cane, and the like is fed into a magazine ahead of a steam pressure chamber in which is housed a rotary device for reducing the material to pulp in a steam environment and particularly in the absence of suspending water. Beyond the defibering chamber there is an outlet device having in series alternately operating valved orifices. By this device, one orifice discharges from the machine while the other orifice is closed. The fiber trapped between the valves is discharged from the intervalve space by the expansion of the high temperature steam also trapped in said space. As originally taught and disclosed the said device discharges the fiber into water.

In applying the Asplund machine to other uses, wherein it became desirable to dry the fiber directly, the discharged fiber was carried by a belt-type conveyer to a suitable drier device which happened to be located at some distance from the machine and at a considerable height above it.

One object of the present invention is to provide means to carry the discharged fiber from the machine for considerable distances away from and even to a higher level, without the use of mechanical means and power to convey the fiber.

In particular, it is an object of the invention to utilize the pressure of the discharged steam to convey the fiber for long distances with or without elevation.

It is still a further object of the invention to provide a cyclone system at the end of said conduit for separating fiber and any steam or gases attendant the discharged material.

A further object of the invention is to provide to said cyclone system a supply of drying gas or air for the removal of water from, or for drying, the fiber in the cyclone system.

It is also an object of the invention continuously to reduce lignocellulose raw material, especially wood, to a mass of fibers, and especially dry fibers, with retention of substantially all the solid content of the original material, and with change in the content of the original material so that it presents less resistance to certain treatments by water, chemical solutions and other reagents, where it is desired to use the fiber as a starting point to produce fibers lacking in some of the solid content of the original wood other than its alpha cellulose content.

Various other and ancillary objects and advantages of the invention will become apparent from the following description and explanation of the invention, as illustrated by the accompanying drawing in which:

2

Fig. 1 represents a plan view of a machine according to the Asplund U. S. Patents No. 2,008,892 and No. 2,145,851.

Fig. 2 represents a conduit and a cyclone system attached to the machine and used to separate steam and gas from the fiber as formed, and used also to dry the fiber.

The apparatus not only provides economy in power and convenience in handling, but may give desirable processing to the fiber. It is a stated objective of the Asplund patent and its process Patent No. 2,008,892, to minimize the time of exposure of the material to the elevated temperatures used in forming the fiber. In connection with other developments employing forming conditions as they exist in the said Asplund machine, I have found that it may be desirable to expose the material, and especially the formed fiber, to elevated temperatures, and particularly to steam, for a much longer time than is permitted by normal operation of said machine.

By employing a long conduit, I have discovered that a back pressure may exist continuously in the conduit at the discharging orifice of the machine. This is reduced as the body of fiber carried in the conduit moves on toward the discharge end into the atmosphere or other receiving space of pressure lower than that in the defibering machine. Of course, the length of this pressure zone in the conduit is dependent in part upon radiation from the conduit, which may be controlled by insulation or its heat surroundings, or both. Where the gas pressure ceases to exist in the conduit the fiber is moved along as a column by mechanical pressure from that portion of the fiber which is moved by the gas pressure.

It is of course to be understood that there are many factors involved which anyone skilled in the art will naturally be obliged to consider in installing or operating the apparatus. Friction of fiber with the conduit, weight of the column of fiber to be lifted, and the existing moisture of added condensate, are all forces opposing the pressure. With these opposition forces also must be considered the loss of pressure in the gas or steam as a result of its expansion or its cooling.

However, in spite of all these oppositions, I have found that a conduit in diameter the same as the machine orifice, say 6 inches, may extend for 150 to 200 feet and at the same time elevate the fiber by as much as 50 feet, the conduit discharging into air from a defibering pressure of 150 lbs. per sq. in. steam pressure. Such distances readily accommodate various pieces of equipment in a plant, at different levels, and at remote locations, to simple connection by a conduit to a fixedly located defibering machine, whereby a plant is made flexible, and whereby a defibering machine may be operated to produce and discharge fiber for various processes of utilization.

The exposure of raw material to the steam in

the machine continues for such a short time, that the chemical reaction in the machine is limited. I have found for example, that by extracting fibers of raw aspen not at all preheated, using 2% fiber consistency in water for two hours, the water soluble extract is about 4% to 5% of the dry wood used. Using fiber defibered in the Asplund machine at 135 lbs. pressure of steam, and immediately exposed to the atmosphere, the water-soluble content is about 10%. I have also determined that prolonged exposures to steam will bring the like water extract to about 27% as a practical limit. By use of the conduit as a steam chamber I may control water solubles to various degrees, in the case of aspen, between substantially 10% and 27%. I have also found that high temperatures and short times can produce as much water-extract as a certain combination of lower temperature and longer time, there being less darkening of the fiber at the latter condition. Hence, for prolonging the steam effect it is desirable to use a lower temperature than exists in the Asplund machine. The discharging valve structure of the Asplund machine is an excellent pressure reducing device for such purpose, and the lengthy conduit is an excellent means for prolonging the time of exposure.

In Fig. 1, an Asplund machine is illustrated in part, showing the essential parts.

A tubular chamber 10 is used to introduce wood as chips, or other lignocellulose material into a high pressure environment within the machine. The inlet 10 has a serrated or notched interior wall which acts to prevent steam pressure pushing back a plug in the inlet formed of the raw material by the action of a ram or plunger 11, acting on raw material fed into the path of the plunger through a hopper opening 12 (Fig. 1) under a hopper 13 (Fig. 2). The inlet 10 opens into a magazine 14 capable of holding high pressure steam therein. The bottom of the magazine connects by a passageway 15 having a screw conveyor 16 therein, operated on the axis 17, by power connection 18. The conveyor feeds the raw material to the center of opposed grinding disks 20 and 21. Disk 20 is stationary and receives the raw material near its center. Disk 21 rotates at high speed on axle 22, driven by a powerful belt connection 23. Means (not shown) permits adjusting the spacing between the disks. A housing 24 for the grinding disks opens to an outlet connection 25. Steam is fed from a supply 26 to a distributing system 27 for introducing the steam into various inlets to the spaces within the machine.

The outlet 25 is connected to an offset extension fixture 28 with valves 30 and 31 at its ends. The valves are arranged to have parallel operating stems 32 and 33, and mechanism (not shown) so operates them that when one is closed or substantially so the other is open or substantially so, as indicated by stressed arrows 34 and 34\*. These reciprocate rapidly and in operation, first admit steam and fiber into the fixture 28, then at least partially close the fixture at the machine end while opening at the other end to discharge the fiber. The degree of opening of the valves and the timing is adjustable, in order to control the amount of steam pressure accompanying the fiber to move it along as described below.

The discharge end of fixture 28 is connected by elbow 35 to an extending conduit 36, shown in Fig. 2 only in cross-section, indicating its vertical extent, better shown in Fig. 2. This may run for long distances horizontally and vertically, and

be branched and valve-controlled. To avoid plugging by the body of fiber moving therein, sharp angles are avoided, as represented by sweeping bends 40 and 41. A Y fixture 42 and valves 43 and 44 are shown, as of the gate type. These may be opened readily, but for closing, the supply of fiber may be stopped until the valve is cleared by the end of the moving fiber. Branch 45 leading from valve 43 represents a supply to any use. Branch 46 leading from valve 44 represents connection to a cyclone or cyclone system.

In the machine, some slight amount of gas is generated from reactions in the wood at the temperature of the steam, and it is desirable to discharge these. This is permitted by any simple cyclone to separate the fiber from the gas and also any residual steam, the discharged fiber being moist. Where moist fiber is useful, it may be taken from such a simple cyclone. However, for the purpose of producing dry fiber, the first cyclone is made a part of a cyclone drying system as now described.

A plurality of cyclones is used, the number being dependent upon design to effect ultimately a dry fiber. Four are illustrated and designated 50, 51, 52 and 53. Conduit 46 enters the top of cyclone 50 which discharges gas and steam to the atmosphere at 54. The bottom of cyclone 50 has alternative outlets, merely for the purpose of illustration. Outlet 55 represents the path for removing moist fiber, and a valve 56 is shown to cut off such outlet. The other outlet is associated with the cyclone system as follows:

Cyclone 50 drops the fiber into a housing 57 in which a vaned rotor 58 operated by motor 59, drops the fiber into a conduit 60 supplied by hot gas from a supply main 61. Fiber and hot air are thus led into a fan housing 63 which blows it through conduit 64 into cyclone 51. The cyclones 51 and 52 continue the series in the same way by like equipment, with some parts indicated as follows: hot gas conduits 65 and 66, fans 67 and 68, fan-outlet conduits 69 and 70. Conduit 70 leads into cyclone 53, which drops dry fiber into a receiver 71.

Where the fiber is useful dry, a high yield is obtained from wood or the like with substantially all the solid substance preserved, as described in my copending application U. S. Serial No. 227,338, now abandoned, filed August 29, 1938, of which the present invention is a continuation in part.

Where the fiber is to be used as a raw material for a solvent extraction, the moist or the dry fiber may be used for extraction by an aqueous solvent.

The extent to which the fiber is subjected to steam (see my copending application U. S. Serial Nos. 351,041 to 351,065, filed August 3, 1940, and related cases), influences the content of extractable matter and the character of the fiber composition. By design and operation as above described, the extent of time and exposure to steam, may be controlled, for such fiber-constitutional purposes, making the apparatus one of chemical as well as physical processing significance, as set forth in the appended claims.

I claim:

1. Apparatus for continuously producing fiber comprising in combination, a high pressure chamber for containing steam under pressure, means to feed high pressure steam into said chamber at a temperature to effect softening of lignocellulose in said chamber, rotary defibering means in said chamber, feeding means to feed lignocellulose vegetable matter into said chamber for de-

fiberizing by said defibering means, said feeding means being arranged and constructed to prevent the exit of steam from said chamber, pressure-reducing means operated to open intermittently in rapid succession for providing an outlet from said chamber for steam and fiber, whereby small batches of loose fiber are discharged in rapid succession, and an open-ended conduit connected to and extending from said pressure-reducing means for containing fiber and steam under pressure and for conveying the fiber, said conduit having a length and cross-section which together are such as to permit said pressure-reducing means to effect a reduction in pressure and to cause a back pressure of steam in said conduit increasing from the open and discharge end of said conduit to said outlet of said chamber, whereby said pressure-reducing means freely discharges fiber into said conduit and into an atmosphere of steam under a pressure which effects movement of the said small batches of fiber along the conduit to said discharge end while exposing all the fibers thereof to the steam in said conduit for a period of time during traverse of the conduit, the length of said conduit further being such that the time of exposure of fibers in said conduit to steam is longer than the time of exposure of lignocellulose to steam in said chamber.

2. Apparatus for continuously producing fiber comprising in combination a high pressure chamber for containing steam under pressure, means to feed high pressure steam into said chamber at a temperature to effect softening of lignocellulose in said chamber, feeding means to feed lignocellulose vegetable matter into said chamber to be defibered, said feeding means being arranged and constructed to prevent the exit of steam from said chamber, rotary defibering means in said chamber, means within said chamber to feed said lignocellulose to said defibering means, pressure-reducing means operated to open intermittently in rapid succession for providing an outlet from said chamber for steam and fiber, whereby small batches of loose fiber are discharged in rapid succession, and an open-ended conduit connected to and extending from said pressure-reducing mean for containing fiber and steam under pressure and for conveying the fiber, said conduit having a length and cross-section which together are such as to permit said pressure-reducing means to effect a reduction in pressure and to cause a back pressure of steam in said conduit increasing from the open and discharge end of said conduit to said outlet of said chamber, whereby said pressure-reducing means freely discharges fiber into said conduit and into an atmosphere of steam under a pressure which effects movement of the said small batches of fiber along the conduit to said discharge end while exposing all the fibers thereof to the steam in said conduit for a period of time during traverse of the conduit, the length of said conduit further being such that the time of exposure of fibers in said conduit to steam is longer than the time of exposure of lignocellulose to steam in said chamber.

3. The method of continuously producing fiber which comprises continuously introducing lignocellulose material to be defibered into a pressure chamber, continuously defibering said lignocellulose mechanically in the presence of steam in said chamber and in the absence of a suspending quantity of water at a temperature above 212° F. and at which the lignocellulose becomes softened to permit ready defibration, while substantially

continuously discharging steam and fiber from said chamber into an elongated laterally confined space and reducing the pressure of the steam at said discharge, while continuously moving said fiber along said space and discharging said fiber from said space by the reduced pressure of said steam into a region of pressure still lower than said reduced pressure, and while employing the length of said space to create a pressure of steam increasing in the direction from said region to said chamber, whereby thermal action in the presence of steam is effected on all the fiber in said space to alter its composition as it moves along said elongated space.

4. The method of continuously producing fiber which comprises continuously introducing lignocellulose material to be defibered into a pressure chamber, continuously defibering said lignocellulose mechanically in the presence of steam in said chamber and in the absence of a suspending quantity of water at a temperature above 212° F. and at which the lignocellulose becomes softened to permit ready defibration, while substantially continuously discharging steam and fiber from said chamber into an elongated laterally confined space and reducing the pressure of the steam at said discharge while continuously moving said fiber along said space and discharging said fiber from said space by the reduced pressure of said steam into a region of pressure still lower than said reduced pressure, and while employing the length of said space to create a pressure of steam increasing in the direction from said region to said chamber, whereby thermal action in the presence of steam is effected on all the fiber in said space to alter its composition as it moves along said elongated space, the time of exposure of the fiber to steam at the reduced pressure in said space being longer than the time of exposure of the lignocellulose to steam at the higher pressure in said chamber.

5. The method of continuously producing fiber which comprises continuously introducing lignocellulose material to be defibered into a pressure chamber, continuously defibering said lignocellulose mechanically in the presence of steam in said chamber and in the absence of a suspending quantity of water at a temperature above 212° F. and at which the lignocellulose becomes softened to permit ready defibration, while substantially continuously discharging steam and fiber from said chamber into an elongated laterally confined space and reducing the pressure of the steam at said discharge, while continuously moving said fiber along said space and discharging said fiber from said space by the reduced pressure of said steam into a region of pressure still lower than said reduced pressure, and while employing the length of said space to create a pressure of steam increasing in the direction from said region to said chamber, whereby thermal action in the presence of steam is effected on all the fiber in said space to alter its composition as it moves along said elongated space, the time of exposure of the lignocellulose to steam in said chamber being insufficient to complete formation of water-soluble material which results from the action of said steam, and the time of exposure of said fiber to steam at the reduced pressure in said space being longer than the time of exposure of the lignocellulose to steam at the higher pressure in said chamber.